

May 27, 1952

R. BROWN

2,598,498

ENAMEL COATED ARTICLES AND METHOD OF MAKING SAME

Filed Sept. 10, 1948



INVENTOR:  
RALPH BROWN  
BY HIS ATTORNEYS  
HARRIS, KIECH, FOSTER & HARRIS  
By 

## UNITED STATES PATENT OFFICE

2,598,498

ENAMEL COATED ARTICLES AND METHOD  
OF MAKING SAME

Ralph Brown, Fall Brook, Calif., assignor to Electrical Products Corporation, Los Angeles, Calif., a corporation of California

Application September 10, 1948, Serial No. 48,708

7 Claims. (Cl. 117—129)

1

This invention relates to an enamel coated article and a method of producing the same. Specifically, the invention pertains to panels capable of being secured together in side-by-side and end-to-end relationship to produce a multi-panel unit suitable for structural purposes, for tiling, or as a background for a sign structure, the present concept relating particularly to a method of coating the outer surfaces of the panels with vitreous enamel in a manner such that no enamel is present on the contacting edges of abutting panels so that cracking or fracture of the hard coating, due to compression between the panels during the assembly of the latter, is entirely avoided.

Metal panels are used quite extensively in the manufacture of signs, the panels being assembled upon a framework and secured to the framework by bolts passing through holes in the panels. It is customary to coat the outer surfaces of the panels with paint, lacquer, pigmented enamel or other protective and ornamental coating agent of suitable color so as to protect the sign from the elements and to afford an attractive appearance. When a more durable and glossy finish is desired, one or more coatings of porcelain or vitreous enamel may be applied to the sign panels and while this is frequently done, much difficulty is experienced due to the fragility of the porcelain coating, especially when the heads of the attaching bolts exert pressure against the porcelain coatings around the bolt holes of the panels. Such a condition results in breakage of the enamel so that signs incorporating porcelainized panels frequently have defects in the porcelain coatings, particularly adjacent the bolt holes and at corners where the enamel is unable to resist the pressure to which it is subjected by the bolts. Such defects are usually touched up with paint which soon deteriorates, and the defects in the porcelain continue to increase in the same way that cracks in glass continue to extend.

Frequently, when sign faces are required to be larger than is permissible through the use of conventional overlapping sheet metal plates, the edges which are to abut may be provided with flanges disposed at right angles to the plane of the face of the plates or panels and such panel segments may be drawn together by bolts extending through holes in the abutting flanges. In such cases, when the panel segments have been coated with vitreous enamel which, in addition to covering the faces of the panel segments, covers the flanges thereof, the pressure exerted

2

by the attaching bolts in drawing and holding the panel segments together is sufficient to crack or break the vitreous enamel and such fractures or chips extend out along the enameled faces of the panel segments. For this reason, the use of vitreous enamel as a coating on components which must be bolted or otherwise secured together has been heretofore believed quite impractical and, while the practice continues, signs embodying such enamel coated components are usually imperfect as regards their outer coated surfaces, when erected on a building or other support.

It is an important object of this invention to alleviate the condition discussed above by providing a method of coating sign panels, and the like, in a manner such that the vitreous coating is deposited only on the planar surfaces of the panel and excluded from the abutting flanges so that the latter can be secured together without danger of cracking or chipping the enamel coating on the planar surfaces of the panels or along the edges thereof. This object is best attained by providing the intersection of the flange and planar surface of each panel with a relatively sharp edge or corner, and a depression in said surface spaced inwardly from the corner and extending alongside the same. By this provision, the vitreous enamel on the surface of the panel, acting through the phenomenon of surface tension or contractile surface force, acts to draw the enamel adjacent the edge toward the depression so as to prevent flow of the coating over the sharp edge and thus precludes any possibility of the enamel flowing onto and lodging on the side of the flange, particularly during the firing of the enamel coating on the panel.

Another object of the invention is to provide a method of applying a coating of vitreous enamel to panels of the character referred to, such method consisting in applying a bonding agent to the outer substantially planar surface of a panel, applying one or more layers of enamel slip to the bonding agent, preferably by a spraying operation, removing any slip which may have been deposited on the flange of the panel during the spraying step, all the slip then being disposed on said generally planar surface with its edges defined by the sharp corner thereof, and finally applying heat to the slip to cause it to flow and fill the voids. The enamel slip, when fired, provides a continuous extremely hard, impervious and highly ornamental coating, the enamel disposed adjacent the sharp corner being drawn inwardly, due to surface ten-

sion of the enamel, and hardening, usually in the form of a bead located in close proximity to said corner but not extending therebeyond. By this method of coating articles of the character referred to, the enamel coating is confined to an area which does not contact portions of panels or other components so that the possibility of cracking or chipping the vitreous enamel, due to compression thereof between the panels, is entirely avoided.

Another object is to provide an ornamental sign panel capable of being joined to adjacent panels, the panel being preferably cast from metal and of a structural shape capable of sustaining considerable load without distortion and without the aid of separate means.

Further objects of the invention will appear from the following specification and from the drawing, which is intended for the purpose of illustration only and in which:

Fig. 1 is a perspective view of a typical flanged panel adapted for use as tiling or as a component of a sign structure, the outer ornamental surface of the panel being coated with vitreous enamel in accordance with the present improved method;

Fig. 2 is an enlarged cross-sectional view through a portion of the panel, taken on line 2—2 of Fig. 1;

Fig. 3 is a view similar to Fig. 2 but showing the panel joined to a similar panel;

Figs. 4a, 4b and 4c are fragmentary cross-sectional views through an enamel coated panel, illustrating the deleterious condition which may exist when the irregular surface of the panel is coated under certain circumstances, but which condition is desirable and utilized to great advantage in the present method of limiting the application of the enamel coating to areas disposed inwardly of the edge of the panel.

Fig. 5 is a view similar to Fig. 3 but showing the adjoining edges of panels of alternative construction; and

Fig. 6 is a composite cross-sectional view of the adjoining edges of a pair of more or less conventional panels, illustrating the deleterious condition which exists when no provision is made for preventing the coating from flowing over the sides or ends of the panels.

As previously indicated, the present invention is directed to coated panels and other elements which are to be assembled in side-by-side or end-to-end relationship by bolts, rivets, or other fastening means. Such elements may take the form of tiles, sign components, the walls of refrigerators, kitchen ranges, etc., the elements 10 illustrated in the present drawing, by way of example, being of a type particularly suitable for use in the construction of outdoor signs and thus will be hereinafter referred to as sign panels.

The sign panels 10 are preferably cast from suitable metal such as aluminum alloy or other light weight metal, and have a generally planar portion 11 and a perimetrical side wall or flange 12 projecting at right angles to the portion 11. The outer surface of the plate-like portion 11 may be grooved, ribbed or otherwise embellished to provide any pleasing and artistic effect. In the present drawing this surface is illustrated as provided with raised bosses or "pillows" 13 which may be of any desired cross-sectional contour, it having been determined that such a pillow'd surface provides an abundance of light-reflecting surfaces which cooperate in diffusing light emanating from the electric illuminating means

of the sign or from adjacent signs or other light sources. The flanges 12 of the panels have apertures 14 through which attaching bolts 15 are adapted to pass, as shown in Fig. 3, nuts 16 being screwed onto the bolts to draw the flanges of adjacent panels together so as to maintain the panels in side-by-side and end-to-end relationship and thus build up a complete sign or building wall of desired size and configuration.

As previously pointed out, it is highly desirable that the exposed surfaces of the sign wall be coated with a material of suitable color which is hard, impervious and durable over long periods of time. A coating material possessing all of these desirable characteristics is vitreous enamel which is well recognized as a highly efficient coating material for elements which are to be exposed to variable weather conditions and which must be of highly ornamental character. Since the development of a vitreous enamel having a relatively low melting point it has become practical to apply such a coating to aluminum alloy articles such as the sign components disclosed herein.

In Fig. 6 there are shown the adjoining sides of a pair of panels, or similar elements 20 which, for the purpose of illustration, may be considered as of the construction thus far described. To apply a vitreous enamel coating 21 to the outer planar surface 22 of the panels, the surfaces are first provided with a suitable bonding agent, after which the enamel "slip" is superimposed on the agent. The slip is usually sprayed thereon and during this operation it is apt to be inadvertently applied to the outer surfaces of the flanges 23. In other instances, the slip may tend to flow over the usually rounded corner or intersection between the surface 22 and the flanges 23 and onto the flanges. In any event, it is necessary to remove any slip from the flanges before firing the same. It has been found that when the slip is subjected to heat to provide the flowable vitreous enamel, the latter in spreading out tends to flow from the surface 22, over the rounded corners, onto the flanges 23 as indicated at 24. In some instances, the enamel may merely form a bead 24 which overhangs the intersection of the surface 22 and the flanges 23. It is thus seen that during the firing process, a portion of the vitreous enamel 21 may harden on the flanges 23 or at the corner between the planar surface and the flanges. Consequently, when the panels 20 are bolted together the frangible enamel disposed between the panels is subjected to considerable compression and thus tends to fracture. Since the enamel coating is continuous, it is apparent that cracks or chips occurring in the compressed portions of the enamel may extend to areas of the enamelled surface 22 which are adjacent to the flanges 23, thus impairing the protective quality of the coating and detracting from the appearance of the sign wall. As previously pointed out, to applicant's knowledge, no satisfactory solution to this problem has heretofore been proposed and, for this reason, vitreous enamelled signs have necessarily been of inferior quality.

It is the aim of the present invention to provide a practical solution to the problem discussed above, through a method and means by which vitreous enamel can be applied to sign panels and other elements in such a manner that injury to the glassy coating is entirely avoided during the drawing of the parts together. Referring to Figs. 1, 2 and 3 of the drawing, a flange 12 of the improved sign panel 10 is ground or other-

wise finished on its exterior surface so as to provide a sharp corner 25 at the intersection of the flange 12 and the planar portion 11.

Spaced inwardly from the sharp corner 25 and extending parallel therewith is a depression 26. The upper surface 27 of the portion 11 that lies between the depression 26 and the corner 25 may slope downwardly from the corner so that the included angle of the corner is made slightly less than 90°. This area 27 of the upper surface of the plate-like portion 11 provides one side of the depression 26, the other side of the depression being preferably formed by the sloping side 28 of the outermost pillows 13 of the panel. The depression 26 provides, in effect, a trough, groove or channel into which a quantity of vitreous enamel can flow. The forming of the sharp corner 25 and the depression 26 at the edges of the panel comprise important steps in the overall method of forming the enamel coated surface of the panel or similar article. With a panel 10 thus fabricated, the outer surface of the plate-like portion 11 is coated with vitreous enamel in the manner to be next explained.

An essential step in the method of coating the exposed surface of the metal panel 10 is that of applying to that surface a suitable bonding agent. Various agents can be advantageously employed for this purpose, and the invention is, therefore, not limited to the use of any particular material. After the bonding agent been applied to the surface to be coated, a layer of semi-fused glassy substance 30, commonly referred to as "enamel slip" is applied in a liquid state to the bonding agent by a spraying or other operation. Following the deposition of the slip, any of the coating material which may have been inadvertently applied to the outer surface of the flange 12 is wiped off so as to confine the material to the surface 11 which is to be coated.

After the bonding agent and slip have been applied in the manner explained above, the slip is exposed to a heating or firing process which, as is well known in the art, changes the characteristics thereof in a manner such that a flowable vitreous enamel is produced. As the coating material 30 which has a low melting point is fired, it spreads out evenly over the entire area to be coated, and during this flowing the glassy material which is disposed on the surface 28 exerts an upward pull on the enamel tending to withdraw the same from the depression 26. Due to this condition, the enamel on the surface 27 is drawn toward the depression 26 and thus prevented from flowing over the corner 25, the material then hardening in this condition and becoming tenaciously bonded or fused to the metallic surface. The prevention of the flow of the vitreous material over the corner 25 is, as above explained, attributed to the phenomenon of surface tension or the contractile surface force due to liquification of the material during the firing process. This results in the formation of beads at the edge of the enamel as shown in Figs. 2 and 3 adjacent the sharp, acute-angled corners 25.

The basic principle upon which the present method of applying enamel coatings to sign panels, or the like, is dependent, is illustrated more or less diagrammatically in Figs. 4a, 4b and 4c. In coating the irregular outer surface 34 of a panel 35 having a groove or flute 36 in the outer surface, the vitreous enamel is applied to the surface including the sides 37 and bottom 38 of the groove and thereafter fired to cause

the enamel to harden thereon. When the bottom 38 of the groove 36 is relatively wide, the vitreous enamel 39 clings to and hardens in place against the bottom and is not affected to any appreciable extent by the upward pulling force exerted by the shrinking of the enamel on the sloping sides 37 of the groove. However, it has been determined that if the width of the bottom 38 of the groove 36 is made relatively small, for example, equal to or less than approximately eight times the thickness of the applied enamel coat, during the firing process the surface tension and shrinking of the enamel on the sloping sides 37 causes pulling forces to be exerted in oppositely inclined directions and thus the enamel is drawn upwardly away from the bottom 38 as shown at 40 in Fig. 4a. During this action, the enamel separates or breaks apart and "crawls" up or, in other words, is drawn upwardly along the sides 37 of the groove 36, as indicated in Fig. 4b, thus causing discontinuity of the enamel surface within the groove and impairing the protective properties and the appearance of the coating.

The principle involved in drawing the enamel upwardly from the bottom of the narrow groove and causing the same to break apart, while ordinarily leading to an inferior coating of the surface of the panel, is employed in my method to great advantage. It has been recognized that since the pulling force of the enamel being fired is capable of withdrawing the enamel from the bottom of the groove and causing it to break apart, this force can be advantageously employed for withholding the enamel coating from flowing over the edge and onto the flange of a sign panel or similar article. It will be seen, by reference to Fig. 4c, that if the panel 35 is cut into two parts by a vertical parting line 43 extending through the center of the groove 36 then the broken edges of the enamel coating are drawn away from this line. The intersection of the line 43 and the bottom surface 38 of the groove 36 may be regarded as the equivalent of the corner 25 of the present panel 10 and it is thus apparent that during the firing of the enamel coating the latter can be caused to draw away from the corner to a slight extent or at least prevented from flowing over the corner, the extent of withdrawal depending largely upon the surface tensions of the heated vitreous enamel. It is thus apparent that the deposition of the enamel coating can be controlled with a high degree of accuracy and the coating prevented from flowing onto areas where it might be subjected to compression when the panels are bolted together.

Several factors contribute to the successful coating of the external surface of a panel of the type referred to above. For example, by sloping the surface 27 toward the depression 26, the contractile surface force, and therefore the upward pulling force, is augmented by gravity when the enamel is fired in a horizontal position. Moreover, by making the corner relatively sharp, the coating material, when in a freely flowable state, will not tend to flow over this corner but rather will be retained by the material on the surface 27. In other words, the sharp corner 25 offers resistance to the flow of material down the side of the flange 12 and, since passage of the material over the corner is prevented, the gravitational force which might otherwise overcome the surface tension of the liquid material is ineffective and the enamel remains on the upper surface

of the panel. It is thus seen that only the desired surface, that is, only that surface which is exposed to view and to the weather, is coated with the vitreous enamel and the flanges 12 remain free from undesirable coating. Consequently, when two panels are drawn together by the bolts 15 and nuts 16 to form a multi-panel wall, the frangible glassy material is not subjected to compression and thus is not damaged.

It has been determined by research that the width of the depression and the distance between its innermost side and the corner 25 is also quite important to the success of the method. This distance, which is represented by the dimension character X in Fig. 2, is preferably not less than one-half the total thickness of the enamel and not greater than approximately four times the thickness of the applied coat, this range permitting the use of enamel of various thicknesses and viscosities. As an example, when the thickness of the enamel is approximately .008 inch, the dimension X may be within the range of .004 inch, depending upon the viscosity of the heated vitreous enamel to be applied. It is thus seen that the width of the surface 27 is extremely important to the success of the method of applying vitreous enamel to articles of the character referred to herein. As will be apparent, when the article to be coated is provided with a pillowed, fluted, ribbed or similar ornamental surface, the channels, such as those indicated at 29' in Figs. 1 and 2, existing between the raised portions intersect the depressions 26 so that the tendency may be for the coating to pull away from the corner 25 to a greater extent adjacent such areas. In such event, the flowable enamel may actually draw away from the adjacent portions of the sharp corner 25 to a degree such that the areas adjacent the edge of the panel may be uncoated and separation or discontinuity of the enamel coating is effected. Consequently, it is highly desirable that the area referred to above be maintained as small as possible. This is accomplished by making the grooves or channels 29' between the ornamental raised portions or the flutes, as the case may be, relatively narrow so as to produce an effective area of a size which will not cause such abnormal pulling force. It has been determined that when the width of the channel 29' is made approximately twice that of the depression 26, a continuous and otherwise satisfactory coating is produced.

It will be apparent that the present method is concerned particularly with coating panels of a cast metal character since the critical dimensions referred to above can best be attained by a casting process. However, it is within the concept of my invention to provide panels fabricated from sheet metal although in such case it is necessary to perform an additional step, that is, to grind the outer surfaces of the flanges so as to avoid rounded corners at the intersection of the flanges and the substantially planar surfaces of the panels.

Referring now to Fig. 5, the invention further contemplates the provision of a panel 50 of alternative construction. In this panel, the corner 51 occurring at the intersection of the planar surface 52 and the flange 53 is made relatively acute by extending the material in a steep ridge. The inclined sides of the ridge and the surface 52 provide between them a depression or channel 54 toward which the vitreous enamel coating is drawn to form beads, as shown, under the influ-

ence of surface tension of the enamel on the surface 52 during the firing of the coating on the panel. Thus, the coating is prevented from extending over the edge of the panel onto the flange 53. Consequently, when the panels 50 are secured together in the relation shown in Fig. 5, there is no tendency to damage the protective and ornamental coating of vitreous enamel.

While I have herein described the improved enamel coated article as embodied in two forms of construction, and the method of applying the enamel coat as comprising a specific series of steps, it will be apparent that various modifications might be made in this construction and method within the concept of the invention. Consequently, I do not wish to be limited in this respect, but desire to be afforded the full scope of the appended claims.

I claim as my invention:

1. In a process of coating a metal article with vitreous enamel wherein said article has a top surface and a side edge portion and is adapted to be assembled in side-by-side abutting relationship with the side edge portion of a similar article to form a panel structure and in which the top surfaces only are provided with a vitreous enamel coating whereby the panel structure has an apparent continuous vitreous surface, the steps of: forming said article so that said top surface merges with said side edge portion at an acute angle to form a shallow depression adjacent said side edge portion and a sharp corner at the junction of said top surface and said side edge portion; applying a vitreous enamel slip to said top surface; firing said article to cause said vitreous enamel to become flowable; and cooling said article to harden said vitreous enamel, the merging of said top surface with said side edge portion at an acute angle causing said vitreous enamel on firing of said article to recede very slightly from said corner and thus be prevented from flowing over said corner and onto said side edge portion and causing fracture of said enamel when said article is assembled in abutting relationship with another of said articles.

2. In a process of coating a metal article with vitreous enamel wherein said article has a top surface and a side edge portion and is adapted to be assembled in side-by-side abutting relationship with the side edge portion of a similar article to form a panel structure and in which the top surfaces only are provided with a vitreous enamel coating whereby the panel structure has an apparent continuous vitreous surface, the steps of: forming said article so that said top surface merges with said side edge portion at an acute angle to form a depression of a depth less than the thickness of said vitreous enamel and a sharp corner at the junction of said top surface and said side edge portion; applying a vitreous enamel slip to said top surface; firing said article to cause said vitreous enamel to become flowable; and cooling said article to harden said vitreous enamel, the merging of said top surface with said side edge portion at an acute angle causing said vitreous enamel on firing of said article to recede very slightly from said corner and thus be prevented from flowing over said corner and onto said side edge portion and causing fracture of said enamel when said article is assembled in abutting relationship with another of said articles.

3. A fired coated metal article adapted to be assembled in side-by-side abutting relationship with at least one similar article to form a panel

structure having an apparent continuous vitreous surface, said article having a top surface and a side edge, said top surface having a shallow depression formed therein including a surface portion merging with said side edge at an acute angle to form a sharp corner, and a vitreous enamel coating on said top surface extending immediately adjacent to but terminating just short of said sharp corner, whereby fracture of said enamel when said article is assembled in side-by-side abutting relationship with another of said articles is prevented.

4. An article as called for by claim 3 wherein said depression is of a depth less than the thickness of said coating.

5. An article as called for by claim 3 wherein said depression is of a depth less than the thickness of the marginal edge of said coating.

6. An article as called for by claim 3 wherein said side edge comprises a flange member disposed at a right angle to the general plane of said top surface.

7. An article as called for by claim 3 wherein said top surface is provided with a plurality of ornamental projections and in which the walls of said projections nearest said side edge merge with said top surface portion of said depression.

RALPH BROWN.

#### REFERENCES CITED

The following references are of record in the 10 file of this patent:

#### UNITED STATES PATENTS

|    | Number    | Name     | Date          |
|----|-----------|----------|---------------|
| 15 | 152,689   | Robinson | June 30, 1874 |
|    | 2,020,476 | Scott    | Nov. 12, 1935 |
|    | 2,024,077 | Thomas   | Dec. 10, 1935 |

#### FOREIGN PATENTS

|    | Number  | Country | Date          |
|----|---------|---------|---------------|
| 20 | 126,341 | Austria | Jan. 11, 1932 |